

## 1

3,074,858

### METHOD FOR THE PRODUCTION OF ASSEMBLIES COMPRISING TITANIUM

Frank Riding, Widnes, England, assignor to Imperial Chemical Industries Limited, London, England, a corporation of Great Britain  
No Drawing. Filed Mar. 31, 1960, Ser. No. 18,807  
Claims priority, application Great Britain Apr. 15, 1959  
6 Claims. (Cl. 204—32)

The present invention relates to improvements in or relating to a method for the production of assemblies comprising titanium and particularly to a method for the production of assemblies involving contact between titanium and graphite as for instance in an interference fit.

Experiments using a laboratory cell producing chlorine by electrolysis of brine have shown that it would be possible for example to design a titanium rod screw-fitting into a graphite anode or a graphite rod contacting a titanium anode which would be satisfactory with regard to the voltage loss at the metal to graphite contact. Prolonged electrolysis at a high anodic current density has shown furthermore no apparent change in the smooth bright surface of a titanium rod or anode.

Measurements of the electrical contact resistance up to very high contact pressures (3600 lb./in.<sup>2</sup>) have shown however that at a contact pressure of even 3600 lb./in.<sup>2</sup> the titanium-graphite contact resistance is about 2.5 times the graphite-graphite resistance at 25 lb./in.<sup>2</sup>.

Nevertheless in, for instance, the field of chlorine production by electrolysis of brine it would be desirable, for example, to be able to utilise titanium as a substitute for the graphite at present used as current lead-in rods because in titanium there is absence of porosity, it has greater mechanical strength and electrical conductivity, it has high resistance to corrosion by chlorinated brine and wet chlorine gas, and because it has an ability to act as an insulator to an electrolyte whilst, at the same time, it is able to pass current to an electronic conductor.

The object of the present invention is to provide a method of lowering electrical contact resistance between titanium and graphite in assemblies of titanium and graphite.

Experiments have therefore been carried out to measure the titanium to graphite electrical contact resistance at various contact pressures for titanium etched with analytical reagent quality concentrated hydrochloric acid for 4 days, similarly etched followed by rhodium electrodeposition, similarly etched followed by platinum electrodeposition, similarly etched followed by five coats of a paint applied platinum-bearing preparation with the firing of each applied coat at 500° C., and non-etched treated with 20 coats of the same platinum-bearing preparation with the firing of each coat applied at 500° C.

In the following table there is recorded the results obtained for variations of titanium to graphite contact resistance in ohms-cm.<sup>2</sup> with contact pressure at room temperature.

| Contact pressure<br>(lb./in. <sup>2</sup> ) | Graphite<br>to<br>graphite | Titanium<br>to<br>graphite | Etched<br>titanium<br>to<br>graphite | Paint<br>applied<br>platinum<br>on etched<br>titanium<br>to<br>graphite | Paint<br>applied<br>platinum<br>on non-<br>etched<br>titanium<br>to<br>graphite | Electro-<br>deposited<br>rhodium<br>on etched<br>titanium<br>to<br>graphite | Electro-<br>deposited<br>platinum<br>on etched<br>titanium<br>to<br>graphite |
|---------------------------------------------|----------------------------|----------------------------|--------------------------------------|-------------------------------------------------------------------------|---------------------------------------------------------------------------------|-----------------------------------------------------------------------------|------------------------------------------------------------------------------|
| 25-----                                     | 0.00635                    | 0.0620                     | 0.0599                               | 0.0309                                                                  | 0.0358                                                                          | 0.00707                                                                     | 0.00230                                                                      |
| 250-----                                    | 0.00139                    | 0.0333                     | 0.0323                               | 0.0072                                                                  | 0.0196                                                                          | 0.00133                                                                     | 0.00101                                                                      |
| 400-----                                    | 0.00115                    | 0.030                      | 0.0248                               | 0.0054                                                                  | 0.0182                                                                          | 0.00092                                                                     | 0.00080                                                                      |
| 725-----                                    | 0.00089                    | 0.0256                     | 0.0141                               | 0.0038                                                                  | 0.0166                                                                          | 0.00067                                                                     | 0.00057                                                                      |
| 1,000-----                                  | 0.00083                    | 0.0241                     | 0.0101                               | 0.0031                                                                  | 0.0155                                                                          | 0.00054                                                                     | 0.00050                                                                      |
| 1,600-----                                  | -----                      | 0.0215                     | -----                                | -----                                                                   | -----                                                                           | -----                                                                       | -----                                                                        |
| 2,200-----                                  | -----                      | 0.0196                     | -----                                | -----                                                                   | -----                                                                           | -----                                                                       | -----                                                                        |
| 2,900-----                                  | -----                      | 0.0178                     | -----                                | -----                                                                   | -----                                                                           | -----                                                                       | -----                                                                        |
| 3,600-----                                  | -----                      | 0.0159                     | -----                                | -----                                                                   | -----                                                                           | -----                                                                       | -----                                                                        |

## 2

From the above table it is seen that the electrical contact resistance for titanium to graphite are of the same order as for graphite to graphite if the titanium contact surface is etched and then given a deposit, particularly an electrodeposit, of platinum or rhodium.

According to the present invention the method for the production of an assembly in which there is electrical contact between titanium and graphite comprises providing the surface of the titanium to face the graphite with a deposited coating of a platinum metal prior to bringing the titanium and graphite into said electrical contact.

Preferably said surface of the titanium is etched prior to the deposition of the platinum metal. Furthermore, preferably the platinum metal is electrodeposited on an etched surface of titanium.

By the term "platinum" or "a platinum metal" is meant platinum, rhodium, or iridium or an alloy of two or more of these metals.

The term "titanium" includes a titanium alloy consisting essentially of titanium.

By way of example the method of the present invention can be applied to a mercury cell having an anode 17.75 inches long of platinum coated expanded sheet titanium as claimed inter alia in copending U.S. application Serial No. 793,687, filed February 17, 1959, and graphite current lead-in rods. These rods can be connected to the anode of platinised expanded sheet titanium by welding to the titanium face of the anode four titanium cups of for instance 1.240 inches internal diameter which accommodate the graphite lead-in rods by a press or interference fit and which have been provided on their inner surfaces with an electrodeposit of platinum.

By measuring potential drops at various currents the contact resistance has been determined for both machined cups and stamped cups having parallel and slightly converging sides respectively when the inner surface of these cups have and have not an electrodeposit of platinum. The results recorded in the following table are expressed in millivolts per ka./m.<sup>2</sup> anodic current density.

|                  | Cup   | Without<br>platinum | With<br>platinum |
|------------------|-------|---------------------|------------------|
| 45 machined----- | ----- | 120                 | 1.5              |
| 45 stamped-----  | ----- | 12                  | 1.4              |

These values show the marked superiority of the electrodeposited platinum coated titanium to graphite contact as against a titanium to graphite contact and also show that the stamped cup, where the interference is maintained throughout insertion of the graphite lead-in rod, is the better design.

Similar results are obtained on passing the current in the opposite direction (i.e. titanium to graphite) indicating the absence of any rectifying properties.

What I claim is:

1. A method for the production of an assembly in

which there is electrical contact between titanium and graphite which comprises providing the surface of the titanium to face the graphite with a deposited coating of a platinum metal and thereafter bringing the platinum-coated titanium and graphite into said electrical contact.

2. A method as claimed in claim 1 wherein said surface of the titanium is etched prior to the deposition of the coating of a platinum metal.

3. A method as claimed in claim 2 wherein the coating of platinum metal on the etched surface of titanium is effected by electrodeposition.

4. An assembly for the passage of electrical current therethrough, said assembly comprising a body of titanium, a surface of which has a platinum metal coating deposited thereon, a graphite body and means for maintaining said graphite body and said titanium body in electrical contact under pressure directly through said coating whereby the electrical contact resistance between said graphite body and titanium body is decreased.

5. The assembly of claim 4 wherein said titanium member is a cup, the inner surface of which is provided

with said coating and said graphite member is a rod fitted into said cup for electrical contact.

6. In a mercury cell, an anode assembly comprising a body of titanium, a surface of which has a platinum metal coating deposited thereon, a graphite body and means for maintaining said graphite body and said titanium body in electrical contact under pressure directly through said coating whereby the electrical contact resistance between said graphite body and titanium body is decreased.

References Cited in the file of this patent

UNITED STATES PATENTS

|           |              |       |               |
|-----------|--------------|-------|---------------|
| 2,624,772 | Phillips     | ----- | Jan. 6, 1953  |
| 2,631,115 | Fox          | ----- | Mar. 10, 1953 |
| 2,636,856 | Suggs et al. | ----- | Apr. 28, 1953 |
| 2,829,091 | Missel       | ----- | Apr. 1, 1958  |
| 2,873,233 | Schnable     | ----- | Feb. 10, 1959 |

OTHER REFERENCES

"Chemical Age," Jan. 3, 1959, page 9.